

Patented July 10, 1923.

1,461,100

## UNITED STATES PATENT OFFICE.

HARRY H. SMITH, OF NEWARK, NEW JERSEY, ASSIGNOR TO WESTINGHOUSE LAMP COMPANY, A CORPORATION OF PENNSYLVANIA.

### METHOD OF TREATING FILAMENTS FOR INCANDESCENT ELECTRIC LAMPS.

No Drawing.

Application filed December 19, 1917. Serial No. 207,861.

*To all whom it may concern:*

Be it known that I, HARRY H. SMITH, a citizen of the United States, and a resident of Newark, in the county of Essex and State of New Jersey, have invented a new and useful Improvement in the Method of Treating Filaments for Incandescent Electric Lamps, of which the following is a specification.

At the present state of the art, it is well known that a metallic filamentary material, such as molybdenum, tungsten and similar highly refractory metals, unless treated in some manner, will tend to alter internally when raised to a point of incandescence in a lamp, and that the degree of alteration will depend upon such factors as the size of filament, efficiency at which it is operated, length of service, etc. One such form of alteration is manifested in what is commonly known as "sagging", the effect of which is an elongation of the filament, particularly if of the coiled type. This effect or elongation produces a detrimental change in a lamp's efficiency, resulting from increased length of the filament, and further promotes the short circuiting of at least portions of the filament, especially if of the spirally wound type, with the consequent early failure of the same.

It is an object of this invention to so treat a metallic filamentary material as to make it substantially non-sag. The treatment is given to a filamentary body in a coherent or homogeneous state, which body may be formed of tungsten powder pressed into an ingot and sintered to render it workable. The sintering process causes the ingot to shrink and become coherent, thereby conditioning it for subsequent mechanical working or drawing down into filamentary form.

It is a further object of the invention to give this treatment at such steps in the manufacture of a lamp as to practically render it impossible to destroy the structure of the filament resulting from my treatment, by subsequent operation wherein the filament may be heated to a high temperature.

I propose to accomplish the above objects by controlling the crystalline structure of a metallic filamentous substance. I have observed that there is a definite relation

between the grain structure and the sagging and non-sagging properties of a filament. I have further observed that by treating a filament, preferably composed of certain constituents, it is possible to predetermine the crystalline structure of the filament and give it a grain structure which remains substantially fixed or is unaffected by subsequent operations. This treatment contemplates raising the temperature of the filament, by the application of an electric current of a given strength, to what may be termed the "germinative temperature" and maintaining it at this condition for a limited time. The germinative temperature may be defined as the minimum temperature at which two adjacent grains can coalesce to form one large grain provided that this larger grain will have sufficiently increased its power of attack to enable it to absorb adjacent grains which cannot coalesce with each other. The germinative temperature may also be considered as a range existing between two other ranges, the preceding one being called the "inert" temperature range and the one following being termed the "growth" range.

The coalescence or grain growth, i. e., the absorption of certain grains by certain other grains, may be promoted or retarded and the germinative temperature accordingly lowered or raised, by such factors as initial grain fineness, prior plastic deformation, mobility of the grain, etc., and in practicing my invention this must be taken into consideration in determining the treating schedule for any given size or kind of filament.

I have found by experimenting that the crystalline structure requisite to prevent a filament from sagging, is one in which the grain structure is large, the grains being of considerable length and of such a formation as to over-lap or interlace with each other. By over-lapping in this manner the arrangement of grains is such that they tend to support each other and this prevents a sagging of the filament. As stated above, it is possible to subject the filament to a heat treating schedule which will not only control, but produce a crystalline structure having long overlapping grains. It is im-

portant that this treatment be given at a time before the filament is raised to a temperature at which grain growth starts, which naturally varies with the size of the filament.

My treating schedule may be applied to any highly refractory metal, such as tungsten, and influence the internal structure thereof, but as intimated above, more satisfactory results may be obtained if the filamentary material is of a certain consistency. In other words, the filamentary material may be made of such a composition as to be inherently susceptible to my treating schedule and thereby accelerate the formation of a given grain structure when the filament is raised to its germinative temperature. Wire which is especially responsive to my treatment in producing a non-sag structure, forms the subject matter of a pending application of Dr. R. D. Hall, filed December 19, 1917, Serial #207,838, and may contain from 2% to 7% by volume (.25% to 1% by weight) of silica and .1% to .4% by volume (.5% to 2% by weight) of thoria combined with tungsten. The character of this wire forms no part of the present invention and further description thereof is considered unnecessary.

An important factor which must be constantly kept in mind during the manufacture of a lamp embodying a filament treated in accordance with my invention is that at no time prior to the giving the filament the treatment, and subsequent to its drawing, must it be allowed to reach a temperature exceeding its germinative temperature. The degree at which this temperature is reached will depend upon the quality of the wire, and I have found by experimenting that this temperature in the case of the special wire referred to, is approximately 1170° C. In carrying out my invention, I have discovered that best results are obtained in producing a non-sag crystalline structure in the special form of filamentary material mentioned above, by subjecting it in a reducing atmosphere to the following schedule; apply a current 90% of the rating for which the lamp is designed, gradually increase this current until it reaches 130% at the end of one minute's time, and then maintain this latter current strength for a period of one minute after which time it is interrupted. This schedule has been found to give very satisfactory results for all tungsten gas filled lamps above 100 watts, but it is obvious that it is subject to modification in treating different type lamps which may have different type filaments. If a filament which has received the treatment just described is examined under a microscope, it will be seen to possess a crystalline structure in which all grains are of large and of a particular formation, i. e., crystals of con-

siderable length which interlace with each other. When the filament is embodied in a lamp and life tested, it will be found to have a non-sagging quality or property.

While I have described my invention as being practiced in connection with special forms of filament, I wish it understood that in its broadest aspect, it contemplates the induced formation of crystals of definite size and shape, arranged so as to form an interlacing structure with each other, and further that by determining a proper treating schedule, it is my belief that such a crystalline formation may be obtained in any kind of a highly refractory metallic filamentary material.

What I claim as my invention is:

1. The method of treating a refractory metallic filamentary body of tungsten or equivalent metal containing crystal growth directing ingredients, which consists in heat-treating said body according to a predetermined seasoning schedule that will cause the development of crystals having considerable length, so arranged as to overlap or interlace with each other.

2. The method of treating a filamentary body of tungsten or equivalent metal containing auxiliary ingredients to produce a crystalline structure therein, which renders the same resistant to sagging, which consists in heating said filamentary body to its germinative temperature and holding it at said temperature in accordance with a predetermined seasoning schedule.

3. The method of treating a filamentary body of tungsten or equivalent metal containing auxiliary ingredients to produce a crystalline structure therein which renders the same resistant to sagging which consists in treating said filamentary body according to a predetermined seasoning schedule before the temperature of said filamentary body is raised to one exceeding its germinative temperature.

4. The method of producing a non-sagging filament from a filamentary body composed primarily of tungsten and having intimately associated therewith silica and thoria, which consists in heat-treating said filamentary body in accordance with the following seasoning schedule: passing a current about 90% of the rating for which the lamp is designed in which said filament is to be incorporated, gradually increasing said current until its value reaches about 130% at the end of about one minute and maintaining said latter current strength for about one minute and thereafter interrupting said current.

5. The method of producing a non-sagging filament from a filamentary body composed primarily of tungsten and having intimately associated therewith silica and thoria, which consists in heat-treating said filament

tary body in accordance with the following seasoning schedule: passing a current about 90% of the rating for which the lamp is designed in which said filament is to be incorporated, gradually increasing said current until its value reaches about 130% at the end of about one minute and maintaining said latter current strength for about one minute and thereafter interrupting said current, said heat-treatment being conducted in a reducing atmosphere.

In testimony whereof, I have hereunto subscribed my name this 3rd day of Dec., 1917.

HARRY H. SMITH.